

Patented July 28, 1942

2,291,590

# UNITED STATES PATENT OFFICE

2,291,590

## ELECTRODEPOSITION OF METALS

Rudolf Lind, Euclid, William J. Harshaw, Shaker Heights, and Kenneth E. Long, South Euclid, Ohio, assignors to The Harshaw Chemical Company, Elyria, Ohio, a corporation of Ohio

No Drawing. Application March 11, 1940,  
Serial No. 323,380

17 Claims. (Cl. 204—49)

This invention relates as indicated to electrodeposition of metals and more specifically, to a process of and materials for use in the process of electrodepositing nickel characterized in that the resultant nickel plate, as deposited, is both bright and ductile. More particularly, the present invention has to do with new addition agents for producing the above-named desirable characteristics in the nickel plate and which may be used with acid nickel baths of usual composition operating under usual conditions.

In order to properly evaluate the present invention, it is necessary to define brightness and ductility or brittleness, terms used in the old art, but used loosely to describe all degrees of brightness or brittleness.

### BRIGHTNESS

It is obvious that an extremely thin deposit of nickel over a highly buffed surface will appear bright. Bright plates of this type have been made for years and are well recognized in the art. Their limitations are that if the plated article is exposed to the atmosphere or to wear, the plate soon disappears or wears off. A plate thin enough so that it will retain substantially the full brightness of the polished base metal is impractical for use even as a base for the electrodeposition thereover of a protective coating of other metals such as chromium. If a heavier deposit is plated out, the brightness of the highly buffed surface diminishes and a gray or white dull deposit is obtained.

A nickel plate which is thick enough to be practical for use and which is brought without buffing is not only desirable per se, but it is particularly advantageous where it is destined for use as the base for an electrolytically deposited chromium plate, since, if the nickel plate does not require to be polished and buffed, a relatively thin plate gives the same protection as the necessarily heavier gray plate, some of which must be taken off in the polishing to secure the desired brightness. Furthermore, a very considerable saving in time and in cost on the production of plated articles becomes possible, whether with nickel plate per se or with additional chromium finish.

Various so-called addition agents have been proposed from time to time for inclusion in nickel plating baths in order to control or affect the character of the electrolytically deposited metal. One principal objective in such modification of the plating bath has been to increase the brightness or luster of the deposited metal.

Many of these previous nickel plating addition agents have allowed a much heavier deposit of nickel to be built up before the brightness of the base metal was materially diminished. When polished articles are plated in such baths, the

deposit is not truly bright but merely, at best, has the same character as the base metal. The brightness produced by such addition agents may, therefore, be characterized as "brightness diminishing with increased thickness of plate on a polished surface."

Others of these previous nickel plating addition agents have produced a plate which would maintain the brightness of the polished base surface, even though the plate was built up to a substantial thickness. They would not build up any substantial brightness on an unpolished surface and, at best, would only very slowly build up brightness on an unpolished surface when plates of extreme thickness were made. The brightness produced by such addition agents may, therefore, be characterized as "brightness maintaining itself with increased thickness of plate on a polished surface."

The addition agents of the present invention produce a plate that not only maintains the brightness of the most highly polished base metal, irrespective of the thickness of the plate within practical limits, but also increases in brightness with increase in thickness of the plate on an unpolished surface. The brightness produced by such addition agents may, therefore, be characterized as "brightness increasing with thickness of plate on an unpolished surface."

### DUCTILITY

The question of ductility is one of vital concern to the plater. In general, all bright plates are harder and, therefore, more brittle than ordinary dull nickel. When enough of many of the previously employed addition agents was added to a bath to produce a bright plate, the plate was often too brittle for commercial use and yet if less addition agent was used, the plate would not be fully bright. A test for ductility may be made by plating on a non-adherent surface and stripping off the foil and bending it double on itself. A plate .001" thick which will pass this test without breaking is considered to have good ductility. A plate .0005" thick which will just pass this test is considered to have passable ductility. A plate .0002" thick which will not pass this test without breaking is considered to have poor ductility.

The addition agents of the present invention not only produce plates with the highest order of brightness, but also with a high order of ductility as defined by the above scale. This is desirable and essential to the practical use of bright nickel plating.

The principal object of the present invention, therefore, broadly stated, is to provide an improved process of and materials for use in the process of electrodepositing nickel which will not only render the nickel plate desirably bright but

which will also preserve or render the plate desirably ductile.

Other objects of our invention will appear as the description proceeds.

To the accomplishment of the foregoing and related ends, said invention, then, consists of the means hereinafter more particularly pointed out in the claims, the following description setting forth in detail certain approved modes of operation of our process and combination of ingredients embodying our invention, such disclosure constituting, however, but certain of various forms in which the principles of our invention may be used.

Broadly stated, our invention comprises the discovery that by the use in acid nickel electrolytes of a plurality of addition agents respectively selected from certain different classes of compounds, we are able to produce deposits which are superior to those obtainable by the use of addition agents from either one of such classes alone. We find that the addition agents from one of said classes, although characterized by an embrittling tendency, are productive of extreme brightness when used in combination with addition agents from the other class and that addition agents from said other class not only cooperate in the production of brightness but also exert a ductilizing effect in the combination. The use of one addition agent from each class is preferable but a plurality from each class can be used successfully. Our cooperating addition agents are suitable for use in a wide variety of nickel electroplating solutions. We have found them to be very effective in aqueous acid nickel sulfate solutions and aqueous acid nickel chloride solutions. Among the nickel sulfate solutions in which they are effective are aqueous acid solutions of nickel sulfate, nickel sulfate and nickel chloride, nickel sulfate and sodium chloride, nickel sulfate and hydrochloric acid, nickel sulfate and ammonium chloride, nickel sulfate and alkali metal chlorides other than sodium chloride, the chlorides serving to produce good anode corrosion. Our addition agents are effective in nickel chloride solutions with and without nickel sulfate. In each of said solutions it is desirable, although not necessary, to employ boric acid or another suitable buffering agent. We prefer to employ a bath containing nickel sulfate together with a suitable chloride, preferably nickel chloride and a suitable buffer, preferably boric acid. We prefer to employ one or more addition agents from one of said classes in quantity to produce the desired brightness and one or more from the other class in quantity to overcome to a substantial extent the resulting embrittling tendency.

Representative of separate classes of compounds which, when used in combination as above stated, produce improved results, are those classes of compounds which may be identified as (1) aromatic compounds containing the group



$x$  being selected from the group consisting of C, N, S and O, which are soluble in the plating bath to the extent of at least one milligram per liter, and (2) aromatic sulfonates, sulfonamides and sulfimides soluble in the bath to the extent of at least  $\frac{1}{2}$  gram per liter. Since these two classes of addition agents are distinct, they will be discussed separately.

Our invention contemplates, as indicated, the use of aromatic compounds of adequate solubility containing the group



where  $x$  may be N, C, S or O or a group containing one of these as the connecting atom between Ar and Ar'. The connecting atom of the group indicated by  $x$  may carry attached groups as for example, when  $x$  is C, a hydrogen or oxygen atom may be attached, or when  $x$  is S, it may carry a hydrogen atom and a chlorine atom; a nitrogen atom may carry a phenyl and a chlorine group, etc. The bonds shown to each aryl group are ortho to each other and the links connecting the Ar and Ar' groups with N and  $x$  indicate single or double bonds. We do not know with certainty in all cases what type of bond exists but we have made use of materials having the acridine, azine, thiazine and oxazine nuclei. Reference is made to Schultz, infra, for accepted theory of structure of these nuclei, the expression



being intended to indicate them generically. Ar and Ar' may be identical or different. Ar and Ar' indicate aromatic cyclic structures such as, for example, benzene or naphthalene nuclei which carry substituent groups. We prefer to employ compounds carrying one or more amino groups connected to ring carbon. Alkyl amino or aryl amino substituents such as  $-\text{N}(\text{Me})_2$ ,  $-\text{NHMe}$ ,  $-\text{N}(\text{Ph})_2$  and the like also are desirable and may be regarded as amino groups. Compounds containing alkyl, such as methyl, ethyl, etc., halogen, sulfonate, hydroxy and nitro groups may also be used. The substituent groups such as amino groups, including alkyl amino groups, appear to be desirable as such while groups such as the sulfonate and halogen groups, unless needed to improve the solubility, apparently are undesirable or indifferent.

The salts of such of these compounds as are basic, e. g. the chlorides, hydrochlorides, acetates and sulfates are to be preferred to such basic compounds themselves because of their greater solubility. It is essential that these compounds, a single one or a mixture of two or more thereof, be present in the solution to an extent to exert their brightening effect, preferably at least two milligrams per liter.

Some specific examples of compounds suitable for our purpose are as follows, being identified where possible by reference to "Farbstofftabellen" by Gustav Schultz, 7th edition, volume I (1931).

TABLE I

- 65 1. Tetramethyl diamino acridine hydrochloride. Schultz No. 902. (An acridine dye, Rhodamine Orange, or Acridine Orange having the nucleus



70 and carrying for methyl and two amino substituents.)

2. Dimethyl diamino acridine hydrochloride.  
3. Diamino acridine hydrochloride.



Ar and Ar' representing benzene nuclei.)  
4. Diamino diphenazine.



Ar and Ar' indicating benzene nuclei.)

5. Safranine Y. Schultz No. 967. (A mixture of 15  
two dyes of the azine type, i. e. having the nucleus.



6. m-Phenyl diamino diphenylazonium chloride.  
(A compound of the formula



- Ar and Ar' representing benzene nuclei.)  
7. Induline BB and/or Induline R. Schultz No. 30  
984. (Azine nuclei.)  
8. Nigrosine. Schultz No. 986. (Azine nuclei.)  
9. Basic Navy Blue D. Schultz No. 1025. Di-  
methylamino phenonaphthazoxonium chlo-  
ride. Oxazine nucleus.)  
10. Diamino phenoazazine.



Ar and Ar' indicating benzene nuclei.)

11. Lauth's Violet, Diamino diphenazthionium 45  
chloride. Schultz No. 1036. (Thiazine  
nucleus.)  
12. Methylene Blue. Schultz No. 1038. (Tetra-  
methyl diamino diphenazthionium chlo-  
ride.)  
13. Methylene Green B. D. Schultz No. 1040.  
(Tetramethyl diamino nitro diphenazthi-  
onium chloride. Thiazine nucleus.)  
14. Toluidine Blue. Schultz No. 1041. (Dimeth-  
ylamino phenoamino tolazthionium chlo-  
ride. Thiazine nucleus.)  
15. Thionine Blue SO. Schultz No. 1042. (Tri-  
methyl ethyl diamino diphenazthionium 55  
chloride. Thiazine nucleus.)  
16. New Methylene Blue. Schultz No. 1043.  
(Diethyldiamino ditolazthionium chloride.  
Thiazine nucleus.)

17. Thiocarmine R. Schultz No. 1044. (Sodium 60  
salt of sulfonic acid of symmetric diethyl  
dibenzyl diamino diphenazthionium sul-  
fonate; internal sulfonate.)  
18. Brilliant Alizarine Blue G. A. Schultz No.  
1048. (Dimethylamino dihydroxynaphtho-  
phenazthionium sulfonate and/or benzyl  
ethylamino dihydroxy naphtho phenaz-  
thionium sulfonate.)

While the quantity of these substances em-  
ployed is not sharply critical, they are used in 70  
small amounts, that is, amounts of the order  
of 2 to 100 milligrams per liter of the bath, the  
upper limit being determined by their embrit-  
tling effect and in some cases, their solubility.

Most of the specific examples given in Table 75

I are commercial products. There are many  
other members of the same groups, mostly not  
commercial products or not obtainable in pure  
form, which we believe would, if available and  
sufficiently pure, have the same effect. In gen-  
eral, impurities are undesirable.

The compounds which carry at least one amino  
group connected to ring carbon constitute an es-  
pecially desirable subgroup, being in general  
more soluble, of a basic character and more con-  
sistently productive of highly brilliant and uni-  
form deposits.

Among the aromatic amino compounds within  
the scope of our invention, products of the form



20 wherein Ar and Ar' represent benzene nuclei,  
carrying at least one amino group on each ben-  
zene ring but not more than three amino groups  
on either benzene ring and their salts such as  
chloride, hydrochloride, acetate and sulfate are  
of outstanding value from the standpoint of con-  
trol of the operation of the bath and are some-  
what superior in respect to brightening effect to  
the more complex compounds.

The second class of materials, representative  
particular ones of which are employed in combi-  
nation with one or more substances of the first  
class of compounds above identified, may be and  
for the purposes of this specification are des-  
ignated as aromatic sulfon-compounds. These  
materials are capable of cooperating with the  
35 materials of the first class to produce nickel de-  
posits having a high order of brightness accom-  
panied by commercial ductility.

Particular examples which we have found to  
give excellent results are as follows:

TABLE II

1. Alpha-naphthalene mono-sulfonate
2. Beta-naphthalene mono-sulfonate
3. Naphthalene disulfonates
4. Naphthalene trisulfonates
5. Sulfonated naphthalene
6. o-Benzoic sulfimide (saccharin, preferably  
as sodium salt)
7. Benzene sulfonamide
8. Benzene sulfohydroxamic acid
9. p-Toluene sulfonamide
10. o-Toluene sulfonamide

The above named addition agents of this sec-  
ond class, suitably in the form of the sodium or  
the nickel salt, may be used in various quantities  
upwards from 0.2 g./l., however, 5 g./l., or less is  
usually sufficient concentration for best results.  
Larger quantities, within the limits of solubility,  
do no harm.

Specific Example 5 of Table II above is such  
as may be produced by reacting 2 parts of 20%  
oleum on one part of naphthalene at 160° C. for  
two hours, neutralizing the resulting mixture with  
nickel carbonate, filtering and diluting to 26° Bé.

65 Where quantities of "sulfonated naphthalene"  
are referred to hereinafter, it is to be understood  
that the quantity specified represents roughly the  
nickel-naphthalene-mixed-sulfonate content of  
the mixture. Five cc. of the nickel neutralized  
reaction mixture is taken as equivalent to one  
gram of nickel-naphthalene-mixed sulfonates.  
Other mixtures of compounds of the second class  
of materials also are satisfactory.

A conventional aqueous acid nickel bath in  
which the combined use of the two classes of

addition agents will be found to give improved results, as above indicated, consists of:

$\text{NiSO}_4 \cdot 6\text{H}_2\text{O}^{**}$  120-450 grams per liter  
 $\text{NiCl}_2 \cdot 6\text{H}_2\text{O}$  15-75 grams per liter  
 $\text{H}_3\text{BO}_3$  15 grams per liter to saturation  
 Sodium lauryl sulfate\* 0-1.0 grams per liter  
 Current density Up to 60 amperes per sq. ft.  
 pH 1.5-5.5  
 Temperature Room to 170° F.

\* Where this compound is referred to, the material sold under the trade name of "Duponol M. E. Dry" is to be understood. It is sold as the technical compound. Other equivalent surface tension reducing agents may be used instead of Duponol. Preparations known as Tergitol 7 and Tergitol 08, sold by Carbide & Carbon Chemicals Co. and said to be sodium secondary alcohol sulfates, may be used instead of Duponol. The quantities required are of the same order.

\*\* Some heptahydrate is usually present. Where nickel sulfate is used herein in specific examples, this mixture of hydrates is to be understood.

In the above table giving the composition of a conventional bath, sodium lauryl sulfate is added for the purpose of reducing the surface tension in order to prevent pitting of the plate. The sulfates of normal primary aliphatic alcohols, having from 8 to 18 carbon atoms, are a class of compounds preferred for use for this purpose.

The following specific examples will serve to illustrate the invention:

#### EXAMPLE I

Nickel sulfate grams 240  
 Nickel chloride do 37.5  
 Borac acid do 37.5  
 Mixture of ms-phenylditolazonium chloride and ms-o-tolylditolazonium chloride (Safranine Y) gram 0.01  
 o-Benzoic sulfimide (saccharin, sodium salt) grams 2.0  
 Sodium lauryl sulfate do 0.25  
 Water to make liter 1  
 pH 4.0  
 Temperature °C 50  
 Current density amp./sq. ft. 40

#### EXAMPLE II

Nickel sulfate grams 240  
 Nickel chloride do 37.5  
 Boric acid do 37.5  
 Dimethylaminophenonaphthazoxonium chloride (Basic Navy Blue D conc.) gram 0.030  
 "Sulfonated naphthalene" (nickel salt) grams 4.0  
 Water to make liter 1  
 pH 4.0  
 Temperature °C 50  
 Current density amp./sq. ft. 40

#### EXAMPLE III

Nickel sulfate grams 240  
 Nickel chloride do 37.5  
 Boric acid do 37.5  
 Tetramethyldiaminodiphenazthionium chloride (Methylene Blue, extra, conc.) do 0.025  
 "Sulfonated naphthalene" (nickel salt) do 5.0  
 Sodium lauryl sulfate do 0.25  
 Water to make liter 1  
 pH 3.3  
 Temperature °C 60  
 Current density amp./sq. ft. 50

#### EXAMPLE IV

Nickel sulfate grams 240  
 Nickel chloride do 37.5  
 Boric acid do 37.5  
 5 Tetramethyldiaminodiphenazthionium chloride (Methylene Green BD) do 0.025  
 "Sulfonated naphthalene" (nickel salt) do 4.0  
 10 Water to make liter 1  
 pH 4.0  
 Temperature °C 50  
 Current density amp./sq. ft. 40

#### EXAMPLE V

Nickel sulfate grams 240  
 Nickel chloride do 37.5  
 Boric acid do 37.5  
 Rhodamine Orange (or Acridine Orange, 20 Schultz #902) milligrams 25  
 "Sulfonated naphthalene" cc 5  
 Water to make liter 1  
 pH 3.5  
 Current density amp./sq. ft. 40

#### EXAMPLE VI

Nickel sulfate grams 240  
 Nickel chloride do 37.5  
 Boric acid do 37.5  
 30 Nigrosine (Schultz #986) milligrams 100  
 "Sulfonated naphthalene" cc 20  
 Sodium lauryl sulfate gram 0.25  
 Water to make liter 1  
 pH 3.0  
 35 Temperature °C 60  
 Current density amp./sq. ft. 50

#### EXAMPLE VII

Nickel sulfate grams 240  
 Nickel chloride do 37.5  
 Boric acid do 37.5  
 Induline R (Schultz #984) milligrams 25  
 "Sulfonated naphthalene" cc 5  
 Sodium lauryl sulfate gram 0.25  
 Water to make liter 1  
 pH 3.5  
 45 Temperature °C 45  
 Current density amp./sq. ft. 40

#### EXAMPLE VIII

Nickel sulfate grams 240  
 Nickel chloride do 37.5  
 Boric acid do 37.5  
 Lauth's Violet (Schultz #1036) milligrams 25  
 "Sulfonated naphthalene" cc 3  
 Saccharine (soluble, soda salt) gram 0.5  
 Sodium lauryl sulfate do 0.25  
 Water to make liter 1  
 60 Temperature °C 60  
 Current density amp./sq. ft. 40

This application is a continuation-in-part of our co-pending application, Serial No. 217,774, filed July 6, 1938, now Patent No. 2,238,861. This application is also a continuation-in-part of our co-pending applications, Serial Nos. 309,232 and 309,233 filed December 14, 1939, now Patents No. 2,198,267 and No. 2,198,268, respectively, which were in turn continuations-in-part respectively of our applications, Serial Nos. 200,120 and 200,121, filed April 5, 1938.

Having thus described our invention, what we claim is:

1. An electroplating bath comprising an aqueous, acid solution of a nickel electrolyte of the

class consisting of nickel sulfate and nickel chloride, said solution having the capability of producing bright and ductile deposits of nickel, such capability having been imparted thereto by the inclusion therein of cooperating addition agents, one of said addition agents being selected from the class of compounds containing the grouping



where  $x$  is selected from the group consisting of N, C, S and O, and which are soluble in the bath to the extent of at least one milligram per liter and mixtures of such compounds, and the other of said addition agents being selected from the class consisting of naphthalene sulfonates, the single ring aryl sulfonamides and single ring aryl sulfimides and mixtures thereof present in solution in the bath to the extent of at least 0.2 gram per liter.

2. An electroplating bath comprising an aqueous, acid solution of a nickel electrolyte of the class consisting of nickel sulfate and nickel chloride, said solution having the capability of producing bright and ductile deposits of nickel, such capability having been imparted thereto by the inclusion therein of cooperating addition agents, one of said addition agents being maintained in solution in the bath in quantity from 2 to 100 milligrams per liter and being selected from the group of compounds containing the grouping



where  $x$  is selected from the group consisting of N, C, S and O, having requisite solubility to permit such concentration and mixtures of such compounds, and the other of said addition agents being selected from the group consisting of naphthalene sulfonates, the single ring aryl sulfonamides and single ring aryl sulfimides and mixtures thereof present in solution in the bath to the extent of at least 0.2 gram per liter.

3. An electroplating bath as defined in claim 2 further characterized in that said first mentioned addition agent comprises a compound having at least one amino group connected to ring carbon.

4. An electroplating bath as defined in claim 2 further characterized in that said first mentioned addition agent is an azine compound having at least one amino group connected to ring carbon.

5. An electroplating bath as defined in claim 2 further characterized in that said first mentioned addition agent is diamino diphenazine.

6. An electrodeposition bath as defined in claim 2 further characterized in that said first mentioned addition agent is diamino acridine hydrochloride.

7. An electrodeposition bath as defined in claim 2 further characterized in that said first mentioned addition agent is Lauth's Violet.

8. An electroplating bath comprising an aqueous, acid solution containing nickel sulfate and nickel chloride, said solution having the capability of producing bright and ductile deposits of nickel, such capability having been imparted thereto by the inclusion therein of cooperating addition agents, one of said addition agents being maintained in solution in the bath in quantity from 2 to 100 milligrams per liter and being selected from the group of compounds containing the grouping



where  $x$  is selected from the group consisting of N, C, S and O, having requisite solubility to permit such concentration and mixtures of such compounds, and the other of said addition agents being selected from the group consisting of naphthalene sulfonates, the single ring aryl sulfonamides and single ring aryl sulfimides and mixtures thereof present in solution in the bath to the extent of at least 0.2 gram per liter.

9. An electroplating bath as defined in claim 8 further characterized in that said first mentioned addition agent comprises a compound having at least one amino group connected to ring carbon.

10. An electroplating bath as defined in claim 8 further characterized in that said first mentioned addition agent is diamino diphenazine.

11. An electrodeposition bath as defined in claim 8 further characterized in that said first mentioned addition agent is diamino acridine hydrochloride.

12. An electrodeposition bath as defined in claim 8 further characterized in that said first mentioned addition agent is Lauth's Violet.

13. The electroplating bath as defined in claim 1 wherein the second mentioned addition agent is an ortho benzoic sulfimide (saccharine, soluble saccharine).

14. The electroplating bath as defined in claim 8 wherein the second mentioned addition agent is an ortho benzoic sulfimide (saccharine, soluble saccharine).

15. An electroplating bath as defined in claim 2 further characterized in that said first mentioned addition agent is diamino diphenazine and said second mentioned addition agent is an ortho benzoic sulfimide.

16. An electroplating bath as defined in claim 2 further characterized in that said first mentioned addition agent is diamino acridine hydrochloride and said second mentioned addition agent is an ortho benzoic sulfimide.

17. An electroplating bath as defined in claim 2 further characterized in that said first mentioned addition agent is Lauth's Violet, and said second mentioned addition agent is an ortho benzoic sulfimide.

RUDOLF LIND.  
WILLIAM J. HARSHAW.  
KENNETH E. LONG.